

## UNITED STATES PATENT OFFICE

2,376,454

## SPHEROIDIZING S. A. E. 2300 SERIES STEELS

Herbert H. Schneider, East Cleveland, Ohio, assignor to The American Steel and Wire Company of New Jersey, a corporation of New Jersey

No Drawing. Application September 21, 1943,  
Serial No. 503,260

1 Claim. (Cl. 148—21.55)

This invention is concerned with spheroidizing steel of the S. A. E. 2300 series, containing from .20% to .45% carbon, the object being to provide the steel, in the shortest possible time, with as good working and forming properties as are obtained by the prior art method of holding the steel slightly below its critical temperature for a prolonged time period.

According to the invention, steel, coming within the defined classification, is heated above its  $A_{e1}$  temperature but not above a temperature causing rapid production of austenite, and is held within this range for a time producing at least some austenite while preserving substantial amounts of pearlite. In this connection, the pearlite may lose its lamellar appearance but substantial amounts of carbides, as microscopically visible undissolved particles, must be preserved.

The next step is to cool the steel at a rate at least as fast as  $25^{\circ}$  F. per hour, and preferably as fast as possible, to within the temperature range where austenite transforms to fine pearlite, bainite, or a mixture of these structures, the steel being held within this range until the austenite, formed during the heating of the steel above its  $A_{e1}$  temperature, transforms. In most instances the steel has sufficient mass so that the cooling is sufficiently slow to directly produce the described transformation, the amount of austenite contained by the steel being restricted, by the need for preserving substantial amounts of pearlite, during the heating above the  $A_{e1}$  temperature.

Summarizing the two preceding paragraphs, the idea is to produce relatively small amounts of austenite in the steel while preserving substantial amounts of its pearlite, and to then quench the steel to transform this austenite to a relatively hard structure, as compared to annealed and spheroidized structures, other than martensite. In all events, care must be taken to avoid the production of martensite. It appears that heating the steel very much above its  $A_{e1}$  temperature favors the production of martensite, and this is another reason for heating the steel to very slightly above this temperature, still another reason being the desire to avoid the rapid production of austenite, so as to provide a relatively extended permissible time during which small amounts of austenite are produced without the loss of too much pearlite, so the invention can properly be carried out in the case of relatively large masses.

The steel, now containing a small amount of hardened structure, in the form of fine pearlite or bainite, and containing a great deal of its original pearlite, possibly altered in form to some extent, is next heated to a temperature range slightly below the  $A_{e1}$  temperature of the steel, and held within this range until spheroidization is completed. During this period, the steel should be

held as close to its  $A_{e1}$  temperature as it safely can without danger of going over this temperature.

The time required for complete spheroidization will be found to be very much shorter than would be expected, yet the steel will have as good working and forming properties as if it had been spheroidized completely by the time honored method of the single step of holding the steel slightly below its critical, it being understood that this old method normally produces better results than can consistently be obtained in the case of most shortened spheroidizing treatments. In many instances, properties obtained by the present invention are better than those obtained by this prior art method.

As a specific example of the invention, S. A. E. 2330 steel is heated to within the range of from  $1210^{\circ}$  to  $1250^{\circ}$  F. and is held within this range for from two to four hours, the steel then being cooled at a rate at least as fast as  $25^{\circ}$  F. per hour to at least  $1050^{\circ}$  F. but not so low as to produce martensite, after which the steel is reheated to within the range of from  $1150^{\circ}$  F. to  $1180^{\circ}$  F. and held within this range for from four to six hours, all as required to effect complete spheroidization. As specific temperatures,  $1230^{\circ}$  F. may be used for holding the steel to slightly austenitize it while preserving its pearlite;  $1000^{\circ}$  F. produces, upon adequately fast cooling, the desired hardened structure; and reheating to and holding at  $1175^{\circ}$  F. results in spheroidization, which occurs rapidly, as compared to other methods, without harm to the properties normally desired of a spheroidized structure.

The necessary determination of the  $A_{e1}$  temperature of the steel may be effected, with sufficient accuracy to carry out the present invention, by austenitizing the steel under question, quenching it violently to render it martensitic, whereby it has a highly stressed, metastable structure, and then reheating the steel to various temperatures, in the vicinity where the  $A_{e1}$  temperature is anticipated, and quenching until the first appearance of untempered martensite in a background of martensite tempered by reheating. The temperature where untempered martensite is first discernible may be taken as the  $A_{e1}$  temperature of the steel.

I claim:

Heating S. A. E. 2300 steel to within the range of from  $1210^{\circ}$  to  $1250^{\circ}$  F. and holding it within this range for from two to four hours, cooling at a rate at least as fast as  $25^{\circ}$  F. per hour to at least  $1050^{\circ}$  F. but not so low as to produce martensite, and reheating the steel to within the range of from  $1150^{\circ}$  F. to  $1180^{\circ}$  F. and holding it within this range for from four to six hours to spheroidize it substantially completely.

HERBERT H. SCHNEIDER.